

# UNITED STATES PATENT OFFICE.

AUGUST LEUCHTER, OF NEW YORK, N. Y.

## ELECTRODEPOSITION OF METALS.

1,026,627.

Specification of Letters Patent.

Patented May 14, 1912.

No Drawing.

Application filed February 15, 1912. Serial No. 677,863.

*To all whom it may concern:*

Be it known that I, AUGUST LEUCHTER, a citizen of the United States, residing at New York, borough of Brooklyn, county of 5 Kings, and State of New York, have invented certain new and useful Improvements in Electrodeposition of Metals, of which the following is a full, clear, and exact description.

10. The invention upon which my present application is based, is an improvement in the art of electrotyping or the production of plate copies by electro-deposition, and resides in a new and useful method or process 15 of effecting the simultaneous deposit of two metals in the form of a composite metal or alloy upon the conducting surface of a mold or other body of which it is desired to obtain a copy or electro.

20. Electrotypes or electros, as is well known, have usually been obtained by the deposition of metallic copper upon the graphitized or prepared surface of a mold or case from which the sheet or plate, when of suitable 25 thickness is stripped. The objections to copper electros, arising from the comparative softness and coarseness of grain of that metal when electrolytically produced, have been fully recognized, but the numerous attempts 30 to produce electros of other and harder metals have usually been attended by failure or at least, with results of doubtful practicability and value.

I have succeeded in producing, electrolytically, printing surfaces and electrotypes generally by the simultaneous deposition of two metals in what appears to be an alloy of both, and which are greatly superior to the ordinary electros, by reason of their 35 hardness, tensile strength, flexibility, fineness of texture and great durability, but in reaching this result I have found that practical success depends upon the maintenance 40 of conditions and the observance of precautions not adopted or followed in previously known processes, and not apparently recognized as essential to the attainment of such 45 results.

In the preferred manner of carrying out 50 my invention I use a tank of the ordinary kind with provision for the suspension therein of the mold or other article upon the surface of which the metal is to be deposited. In conjunction with such mold, and its conducting 55 surface as a cathode, I use an anode

of nickel, and an electrolyte containing an iron salt, preferably sulfate of iron.

It is well understood by those skilled in this art, that certain definite relations of anode and cathode, particularly with respect to spacing, manner of suspension, and surface contact with the electrolyte are necessary for economical and successful operation, and it is of primary importance that all of these should be observed and secured. 60 In addition to this, however, I have found that it is essential to so determine and adjust the resistance of the bath as a whole with respect to the impressed electromotive force of the circuit arbitrarily fixed by practical conditions and limitations, that the effective voltage shall have a value intermediate to the higher voltage necessary for effecting the deposition of nickel, and the lower voltage suitable for the deposition of the 65 iron. These conditions I have found to be obtainable only by using the metal of higher resistance as an anode, and the metal of lower resistance in solution in the electrolyte, and by so making and arranging the 70 anode that its rheostatic effect will reduce the impressed electromotive force to that 75 value. For example, having established in other respects the proper conditions and relations for a given bath, I employ a source 80 of current giving an electromotive force of five volts, and use an anode of nickel having a rheostatic effect sufficient to reduce the electromotive force to three volts, a value 85 somewhat in excess of that necessary for the deposition of iron and somewhat below that ordinarily necessary for the deposition of nickel, but which under the conditions secured by the particular combination under consideration I have found to be capable 90 of effecting the deposition of both metals 95 simultaneously.

It is manifest that in carrying out the process above described, nickel from the anode will go into the electrolyte, although 100 it will not unduly accumulate because of the rate at which it is deposited. It is essential, however, that the iron should at all times predominate in the electrolyte and hence loss of iron by electrolytic action must 105 be compensated for by the addition of fresh solution so as to preserve a substantial preponderance of iron over nickel in the electrolyte. This discovery has proved of the greatest value and importance in the art 110

of producing on a commercial scale, electrotypes of harder metal than copper, for while it is possible to deposit both nickel and iron simultaneously by the use of either

- 5 an iron or a nickel anode in a bath containing nickel or iron respectively in solution, unless the conditions above prescribed are established and maintained, the action is not capable of being prolonged beyond a  
 10 limited time, after which the quality of the deposit deteriorates, by reason of the preponderance of one of the constituent metals in the plate, which may become so great as to result in the deposition of one to the  
 15 total exclusion of the other.

In practice the nickel suitable for anodes is never pure, and its electrical resistance will depend upon the proportion of other metals or impurities present. The production or selection of the proper composition and form of electrode suitable for the purpose of this invention is a matter well within the skill of those versed in the art.

In the above description of my invention the illustration of specific procedure is confined to nickel and iron. These two metals are the ones which I prefer, and their use involves the most typical or characteristic embodiment of the invention, mainly because of the fact that their resistances to decomposition differ so widely. The same conditions obtain and the same rules apply, however, to other metals capable of being electrolytically deposited in the form of alloys, and which require currents of different voltage for their deposition. In all such cases the metal of higher resistance should be used as or in the anode, and by its predetermined rheostatic effect reduce the voltage to a value intermediate to those required or suitable for deposition of either metal alone.

What I claim is:—

1. The improvement in the art of simultaneously depositing two metals electrolytically upon a conducting surface both of which metals are capable of being plated, which consists in using the metal of lower resistance in solution in the electrolyte, forming the anode of the metal of higher resistance and reducing by the rheostatic

effect of the anode the electromotive force of the current to a value intermediate to the voltages necessary and suitable for the deposition of either metal alone.

55

2. The improvement in the art of simultaneously depositing nickel and iron electrolytically upon a conducting surface, which consists in using a nickel anode in an electrolyte containing iron in solution, and reducing by the rheostatic effect of the anode the electromotive force of the current to a value intermediate to the voltages necessary and suitable for the deposition of either nickel or iron alone.

60

3. The improvement in the art of simultaneously depositing two metals electrolytically upon a conducting surface both of which metals are capable of being plated, which consists in using in predominating proportion the metal of lower resistance in solution in the electrolyte, forming the anode of the metal of higher resistance and reducing by the rheostatic effect of the anode, the electromotive force of the current to a value intermediate to the voltages necessary and suitable for the deposition of either metal alone.

65

4. The improvement in the art of simultaneously depositing nickel and iron electrolytically upon a conducting surface, which consists in using a nickel anode in an electrolyte containing iron and maintaining at all times in the electrolyte a preponderance of the iron.

70

5. The improvement in the art of simultaneously depositing nickel and iron electrolytically upon a conducting surface, which consists in using a nickel anode in an electrolyte containing iron, maintaining at all times a preponderance of iron in the electrolyte, and effecting the deposition of the metals by a current of a voltage intermediate to that required for the deposit of nickel alone and that suitable for the deposit of iron alone.

75

In testimony whereof I affix my signature in the presence of two subscribing witnesses.

AUGUST LEUCHTER.

Witnesses:

M. LAWSON DYER,  
B. R. SANDMAN.